# EUROPEAN PATENT SPECIFICATION

(11) **EP 0 459 354 B1**
(45) Date of publication and mention of the grant of the patent: **03.08.1994**
(21) Application number: 91108587.6
(22) Date of filing: 27.05.1991
(51) Int. Cl.: C10M 169/04

(54) **Lubricating oil composition**
Schmierölzusammensetzung
Composition d'huile lubrifiante

(30) Priority: 28.05.1990 JP 137558/90
(43) Date of publication of application: 04.12.1991
(73) Proprietor: NIPPON OIL CO., LTD., Tokyo (JP)
(72) Inventor: Takashima, Hiroyuki, Yamato-shi, Kanagawa-ken (JP)
(74) Representative: Dr. Elisabeth Jung Dr. Jürgen Schirdewahn Dipl.-Ing. Claus Gernhardt

(56) References cited:
- DE-B- 1 039 174
- US-A- 2 590 451
- PATENT ABSTRACTS OF JAPAN vol. 9, no. 218 (C-301)(1941) September 1985& JP-A-60 81 132 (AKIRA WAKAYAMA ) May 9, 1985

## Description

### (1) Field of the Invention

This invention relates to a lubricating oil composition for machineries such as compressors and the like.

### (2) Description of the Prior Art

Compressed air used in association with health, for example, used in food and medicine manufacturing plants or in the instruments for medical facilities, is usually produced by means of a combination apparatus of an oil cooling compressor and an oil mist filter-type compressor. The oil mist filter-type compressor is rarely employed in small and medium-sized manufacturing plants or in medical facilities, because the production costs of compressed air is almost twice the costs of that produced by an oil cooling compressor. These higher costs are due to the fact that the minimum economical capacity is about 15 KW.

Examples of the fields in association with health in which compressed air is utilized include those in manufacture of food such as ice cream for stirring purposes, food treating facilities to skin vegetables such as onions by instantaneously blowing off the skin, breweries of bean paste and the like for stirring purposes, bottling of food such as soft drinks and beverages to blow off overflows, washing of bottles, transportation of powdery matters such as sugar, in portable air drills as an air source and for cleaning the throat for dentistry, and the like.

In case of a combination of an oil cooling compressor and an oil mist filter-type compressor, traces of oil mists, in an amount of several to several tens of ppm, may inevitably leak out of the system because of the difficulty of complete removal of the oil mists in the compressed air over an extending period of time.

Screw-type compressors have been commonly employed for the production of dried ice in medium to large scale plants to compress carbon dioxide. In this case, the lubricating oil used is strictly selected from the group consisting of innoxious lubricating oils in due consideration of being harmless to the human body because said lubricating oil is used under direct contact with the carbon dioxide gas. At the same time, the lubricating oil is further required to have antioxidation properties because a very small amount of air may be mixed in with the carbon dioxide gas.

Therefore, as for compressor lubricating oils for such uses, severely selected and innoxious lubricating oils such as animal and vegetable oils and liquid paraffins have been used. However, animal and vegetable oils and liquid paraffins are insufficient in rust prevention effects and antioxidation properties. Under the existing conditions, it is impossible to find such innoxious lubricating oils on the market which are safe for equipment and have excellent antioxidation properties and rust preventing performances as well.

The present invention is based on finding that a remarkable improvement in performances such as lubrication, rust prevention, and oxidation stability of an innoxious lubricating oil can be attained by incorporation of a specific compound in a specific amount into a liquid paraffin-based lubricating base oil.

### 3. Summary of the Invention

An object of the present invention is to provide an innoxious lubricating composition having improved lubricating properties, rust inhibiting properties, oxidation stability. More particularly, the present invention is to provide a lubricating composition comprising a major amount of liquid paraffin as a lubricating base oil and about 0.01 to 1.0 % by weight based on the total amount of the lubricating oil composition of saturated fatty acids having 12 to 22 carbon atoms as an essential component.

### 4. Detailed Description of the Invention

In the present composition, a liquid paraffin is employed as the lubricating base oil wherein the liquid paraffin having a kinematic viscosity of 7 to 160 cSt at 40 °C is preferred.

An example of preferable liquid paraffins includes a highly refined light lube cut obtained from crude oil by vacuum distillation followed by sulfuric acid treating.

As for the saturated fatty acids having 12 to 22 carbon atoms, natural fatty acids or synthetic fatty acids may be employed, both straight and branched chain fatty acids are usable. Examples of the saturated fatty acids include straight and branched chain fatty acids such as lauric acid, dodecylic acid, myristic acid, pentadecylic acid, palmitic acid, heptadecylic acid, stearic acid, nonadecanoic acid, arachic acid, and mixtures thereof. Among them, C₁₄, C₁₆, C₁₈ or C₂₀ fatty acid, and mixtures thereof are preferred. When saturated fatty acids other than the acids having 12 to 22 carbon atoms or unsaturated fatty acids are employed in the place of the saturated fatty acids having 12 to 22 carbon atoms, performances such as oxidation stability and lubrication are unsatisfactory.

These fatty acids of the present invention have been designated as odorants in the legal definition of the term "food additives" and sorted into one of the standard raw materials used in the production of cosmetics and it is clear that they are perfectly innoxious to the human body. Said C₁₂ to C₂₂ saturated fatty acids are in an amount of about 0.01 to 1.0 % by weight based on the total amount of the composition, preferably about 0.01 to 0.5 % by weight. When the content is less than 0.01, performances such as oxidation stability, rust prevention and lubrication are insufficient, and there is no reward to incorporate the acids in an extra amount beyond the range.

According to the composition aspects of the present invention, a lubricating oil composition having various improved performances may be provided by incorporation of saturated fatty acids having 12 to 22 carbon atoms as an essential component with a major amount of liquid paraffin as the lubricating base oil.

However, dibutyl hydroxytoluene and/or tocopherol (Vitamin E) may be added further to improve the lubricating performances in the present composition.

Examples of Dibutyl hydroxytoluene and/or tocopherol (Vitamin E) include 2,6-di-tert-butyl-4-hydroxytoluene, α-tocopherol, β-tocopherol, γ-tocopherol, δ-tocopherol, and mixtures thereof.

These substances have been also designated as antioxidants in the legal definition of the term "food additives", and are completely harmless to human body.

Dibutyl hydroxytolune and/or tocopherol is in an amount of 0.0001 to 5.0 % by weight, preferably 0.001 to 2.0 % by weight, more preferably 0.001 to 0.1 % by weight based on the total amount of the composition.

In order to further improve the lubricating performances of the present inventon, various other additives may be optionally used, in so far as they are not harmful to the human body.

Examples of such innoxious additives include higher fatty alcohols such as oleyl alcohol, animal and vegetable fatts and oils including their partially hydrogenated products, higher fatty acid esters such as methyl laurate and butyl stearate as an oiliness improver, tert-butyl-hydroxyanisol as an antioxidant, sorbitan fatty acid esters such as sorbitan monooleate, sucrose fatty acid esters such as sucrose monolaurate and the like as a corrosion inhibitor, and mixtures thereof.

Although the amount is optional, these other additives are usually in an amount of less than about 20.0 % by weight respectively, preferably about 0.1 to 10.0 % by weight based on the total amount of the composition, said amount not being limited.

### (Examples)

In order to further illustrate the composition of the present invention, the following examples are provided. It will be understood that the examples as hereinafter set forth are provided for illustrative purposes and are not intended to limit the invention as herein disclosed and as set forth in the claims.

### Examples 1 to 6 and Comparative Example

According to the compositions listed in Table 1, the lubricating compositions (Examples 1 to 6) of the present invention were prepared. Performance tests were carried out for these compositions by the following methods and the test results are set forth in Table 1. A blank test was run with a sample consisting of the same liquid paraffin used as the base oil, and the results are also set forth in Table 1

### (Antiwear test):

According to ASTM D 4172 " WEAR PREVENTIVE CHARACTERISTICS OF LUBRICATING FLUID (FOUR-BALL METHOD)", the wear scratches (mm) of the samples were measured at a speed of 1,200 r.p.m., a load of 15 kg and a duration of 30 minutes.

### (Rust preventing test)

According to JIS K 2510" RUST INHIBITING TEST FOR LUBRICATING OIL", the rust inhibiting performances were evaluated.

### (Oxidation stability test)

According to JIS K 2514 3.3 " OXIDATION STABILITY TEST FOR LUBRICATING OIL BY ROTARY BOMB METHOD", the life times (min.) of the samples in an oxidation atmosphere were measured at a temperature of 120 °C.

As described above, the lubricating compositions of the present invention have improved performances of lubrication, rust prevention and antioxidation, and are completely innoxious to the human body.

## Claims

1. A lubricating oil composition comprising a major amount of liquid paraffin as a lubricating base oil and about 0.01 to 1.0 % by weight based on the total amount of the lubricating oil composition of a saturated fatty acid having 12 to 22 carbon atoms as an essential component.

2. The lubricating oil composition according to Claim 1 wherein said composition comprising further about 0.0001 to 5.0 % by weight based on the total amount of the lubricating oil composition of dibutyl hydroxytoluene and/or tocopherol.

3. The lubricating oil composition according to Claim 1 or 2 wherein said saturated fatty acid selected from the group consisting of C₁₄, C₁₆, C₁₈, and C₂₀ saturated fatty acids and mixtures thereof.

4. Use of the lubricating oil composition according to Claim 1,2 or 3 as compressor lubricating oil.

## Patentansprüche

1. Eine Schmierölzusammensetzung, umfassend eine größere Menge flüssigen Paraffins als ein Grundschmieröl und etwa 0,01 bis 1,0 Gew% einer gesättigten Fettsäure mit 12 bis 22 Kohlenstoffatomen als ein wesentlicher Bestandteil, basierend auf der Gesamtmenge der Schmierölzusammensetzung.

2. Die Schmierölzusammensetzung nach Anspruch 1, wobei die Zusammensetzung außerdem etwa 0,0001 bis 5,0 Gew% Dibutylhydroxytoluol und/oder Tocopherol umfaßt, basierend auf der Gesamtmenge der Schmierölzusammensetzung.

3. Die Schmierölzusammensetzung nach Anspruch 1 oder 2, wobei die besagte gesättigte Fettsäure aus der Gruppe, die aus gesättigten C₁₄-, C₁₆-, C₁₈- und C₂₀-Fettsäuren und deren Gemischen besteht, ausgewählt ist.

4. Die Verwendung der Schmierölzusammensetzung nach den Ansprüchen 1, 2 oder 3 als ein Kompressorschmieröl.

## Revendications

1. Composition d'huile lubrifiante comportant une proportion majeure de paraffine liquide comme huile de base lubrifiante et environ de 0,01 à 1,0 % en poids par rapport au poids total de la composition d'huile lubrifiante, d'un acide gras saturé, ayant de 12 à 22 atomes de carbone, comme composant essentiel.

2. Composition d'huile lubrifiante selon la revendication 1 dans laquelle ladite composition comporte en plus environ de 0,0001 à 5,0 % en poids par rapport au poids total de la composition d'huile lubrifiante, de dibutyl hydroxytoluène et/ou de tocophérol.

3. Composition d'huile lubrifiante selon la revendication 1 ou 2 dans laquelle ledit acide gras saturé est choisi dans le groupe formé des acides gras en C₁₄, C₁₆, C₁₈ et C₂₀ et des mélanges de ces derniers.

4. Utilisation de la composition d'huile lubrifiante selon l'une quelconque des revendications 1 à 3 comme huile lubrifiante pour compresseur.
